

June 4, 1935.

F. HANSGIRG

2,003,487

## PROCESS OF PRODUCING SUBSTANTIALLY PURE MAGNESIUM

Filed Feb. 3, 1933

4 Sheets-Sheet 1



三

Inventor  
Trity Hanging  
by Brown, Critchlow & Fitch  
his attorney.

June 4, 1935.

F. HANSIGRIG

2,003,487

PROCESS OF PRODUCING SUBSTANTIALLY PURE MAGNESIUM

Filed Feb. 3, 1933

4 Sheets-Sheet 2

Fig. 2



Inventor  
Fritz Hansig  
by Brown, Critchlow & Felt  
his attorney.

June 4, 1935.

F. HANSGIRG

2,003,487

## PROCESS OF PRODUCING SUBSTANTIALLY PURE MAGNESIUM

Filed Feb. 3, 1933

4 Sheets-Sheet 3

Fig.3



June 4, 1935.

F. HANSGIRG

2,003,487

## PROCESS OF PRODUCING SUBSTANTIALLY PURE MAGNESIUM

Filed Feb. 3, 1933 4 Sheets-Sheet 4

Fig. 4.



**WITNESSES**

A. B. Wallace.  
F. S. Flick.

**INVENTOR**

Fritz Hanegerg  
by Brown, Bitchler & Klein  
his attorney.

## UNITED STATES PATENT OFFICE

2,003,487

PROCESS OF PRODUCING SUBSTANTIALLY  
PURE MAGNESIUM

Fritz Hansgirg, Radenthein, Austria, assignor to  
American Magnesium Metals Corporation,  
Pittsburgh, Pa., a corporation of Delaware

Application February 3, 1933, Serial No. 655,067  
In Austria February 11, 1932

13 Claims. (Cl. 75—17)

This invention relates to a process of and apparatus for producing substantially pure magnesium.

Like all solid substances having a considerable vapor tension even below their melting point, metallic magnesium displays the tendency to pass directly from the condition of vapor into the solid state, without the occurrence of a liquid phase. It has therefore been repeatedly recommended to purify magnesium by sublimation, or to produce it in crystalline form, from magnesium-containing originating materials, a process which, however, is attended inter alia, with the drawback, in operating on a technical scale, that it can only be performed in a periodic manner. On the other hand, the distillation of magnesium has hitherto encountered serious difficulties.

One object of the present invention is to separate substantially pure magnesium from non-volatile concomitant substances.

Another object of my invention is to enable magnesium to be distilled so as to condense the distillate as a liquid deposit.

A further object of the invention is to provide a process of and apparatus for the distillation of material containing metallic magnesium which can be carried on continuously.

My process comprises passing crude metallic magnesium or material high in magnesium, continuously through a heated zone, in order to heat it to a temperature above the melting point, and preferably in the neighbourhood of the boiling point of magnesium, the disengaged vapors being carried by an inert or reducing gas, through an interposed filter, into the condensing zone, the vapors being prevented from cooling below the solidification point of the magnesium, by being heated on their way to the condensing zone, and being thereafter suddenly cooled to condensation point. The filtration serves to remove contaminating particles of dust from the metallic vapors. This process is performed at reduced pressures.

While various types of apparatus might be employed for carrying out this process, a typical apparatus according to the present invention consists substantially of an externally heated distillation chamber, which is provided with a conveyor and connected, at each end, with lock chambers, through a stock vessel or collector, and also with a condenser from which the molten magnesium runs off into a collector, for example, through a barometric outlet, a filter being interposed between the said distillation chamber and the said condenser. The still, filter, condenser,

outlet and receiver are preferably housed in a common heating chamber, such as an electric radiation furnace.

In order to render the filtration process continuous, it is advisable to employ a filter of loose, granular material, piled up loosely, between an intake and closable outlet, in the passage connecting the still chamber with the condenser.

In a preferred embodiment of apparatus for carrying out the invention, the condenser consists of a hollow body, closed below and internally cooled, and preferably with a curved bottom, said body being disposed in a heated jacket, in such a manner that the incoming vapors bathe the lowest portion of the cooling surface. This cooling tube is preferably provided with a device for maintaining a liquid or gaseous cooling medium in circulation, the arrangement being such that the heat is transmitted through the outer tube to the cooling medium principally by radiation. To enable the cooling action to be accurately regulated, it is advisable to arrange said circulating device so as to be vertically adjustable.

In order more clearly to understand the nature of the invention, reference is made to the accompanying drawings, which illustrate diagrammatically and by way of example, an embodiment of apparatus suitable for carrying out the process of the invention.

In said drawings Fig. 1 shows a front elevation in partial section;

Fig. 2 a cross section;

Fig. 3 a vertical section through a modified embodiment; and

Fig. 4 a detail of a further modification.

Like reference characters denote like parts in the several figures of the drawings.

According to the example shown in Figs. 1 and 2, the distillation chamber 1 is in the form of a tube, which extends through a suitable heating apparatus, such as an electric radiation furnace 2. The material to be distilled is placed in the charging hopper 3 and passes through the lock chamber 4—the closure members 5 and 6 coacting with levers—into a stock vessel 7, from which it is continuously fed, by means of a worm 8 or the like, into the distillation chamber 1, through which the material is conveyed by means of a worm 9 or the like. The residue falls into a collector 10, from which it is discharged through a lock chamber 11, with the closure members 5<sup>a</sup> and 6<sup>a</sup>. The collector 10 and chamber 11, as also the chamber 4 and stock vessel 7, are connected with the vacuum pump by means of pipes adapted to be closed independently.

35

25

30

35

40

45

50

55

55

Midway along its length the distillation tube 1 is connected by a conduit 12 with the outer shell 13 of a condenser, the discharge pipe 14 of which dips into the receiver 15. In the bottom of 5 the receiver 15, there is provided a valve 16. By arranging the condenser at a level more than 6 meters above the outlet level, a perfectly automatic barometric outlet device is obtained. This known arrangement can also be replaced by the 10 known double receiver for vacuum distillation, which enables work to be carried on without interruption by reversing devices.

According to the embodiment shown in Fig. 2, the condenser consists of the cylindrical hollow vessel 17, closed below by a curved bottom and disposed upright in the heated shell 13, in such a manner that the incoming vapors bathe the lowest portion of the cooling surface. A tube 18 is centred in the tube 17 so as to leave a 20 small intermediate space all round and allow the transmission of heat to take place principally by radiation and is cooled by means of a liquid or gaseous cooling medium, which is admitted through the tube 19<sup>a</sup> and passes away through 25 the lateral branch 19<sup>b</sup>. The whole of the circulation device is vertically adjustable in the tube 17, in order to enable the cooling action to be accurately regulated.

In order to remove accompanying dust, a filter 30 is interposed in the pipe 12 connecting the chamber 1 with the condenser 13. The filtering medium consists preferably of loose, granular material, such as sintered magnesite or coal slack, disposed loosely in the connecting pipe. The 35 arrangement shown in Fig. 2 has been adopted to enable the filtering medium to be replenished without interrupting the work. The filtering medium 20 is disposed in a hopper 21, to the lower end of which is attached a tube 23, which can 40 be closed by a valve 22 and dips into a collector 24, whilst a pipe 25, leading from a stock vessel 26, rests on the heap. On the valve 22 being opened, the entire column of material is set in motion, the active portion becoming changed. 45 If desired, the valve can be left slightly open all the time, so that the changing is continuous. Since the filtering medium is more rapidly clogged up on the intake side than on the discharge side, it is advisable to arrange that the changing of 50 the medium does not proceed with the same velocity on the two sides. For this purpose a deltoid member 27 is disposed, slightly eccentrically, in the hopper 21, so that the outlet passage on the intake side of the vapors is wider than the passage on the outlet side, and the medium accordingly moves more rapidly on the intake side than at the outlet side.

In order to direct the flow of the magnesium vapors, they are conducted to the condenser by 60 means of a current of inert or reducing gas, such as hydrogen. For this purpose, supply pipes 28, 29, 30, 31, are employed, which, in the example shown, are attached at both ends of the reaction chamber 1 (Fig. 1) and to the stock vessel 65 26 and outlet pipe 23 (Fig. 2) respectively.

The material to be distilled, such as magnesium dust, furnished by the electrothermal reduction of magnesium compounds, is heated in the heating zone to a temperature—according to the degree of vacuum—at which the magnesium already possesses a high vapour tension, preferably to a temperature near (slightly above) boiling point. The pipe 12 leading to the condenser (Fig. 1), the filter and the shell 13 of the condenser are heated to such an extent that the

internal temperature cannot fall below the solidification temperature of the magnesium. If the distillation be conducted within a pressure range of 50 to 200 mms. mercury gauge, the distillation tube and the other heated members of the device are maintained at a temperature between 850° and 1000° C. The actual cooling temperature of the condenser is between 680° and 800° C. 5

According to the embodiment shown in Fig. 3, 10 the horizontal reaction chamber is replaced by a vertical tube 32, forming the casing of one side of a bucket elevator 33. Before entering the heated portion of the casing 32, the buckets 34 are filled with magnesium-containing material 15 from a stock vessel 35 and this material is thereafter superposed by a filtering material discharged from a stock vessel 37. The outlets of each vessel are adapted to be closed by slides 36, 38 respectively. The vapors generated in the 20 heated section of the tube 32 pass through the filtering medium and are carried off to the condenser 13 by means of the flushing gas admitted at 39 and 40.

In Fig. 4 there is illustrated a double receiver 25 which may be used in connection with the present process, and which is similar to that shown in Ullmann "Enzyklopaedie der Technischen Chemie" of 1929, second edition, third volume, at page 610. It comprises two receivers 45, 45' 30 which may be connected alternatively by means of the three way valve 46 through pipe 14 to the condenser. Each of the receivers is adapted to be connected with the vacuum pump or the atmosphere by means of pipes controlled by valves 35 48, 48' and 49, 49' respectively. The discharge pipes of the receivers 45 and 45' may be closed independently by valves 53 and 53' respectively. Before the distillate is allowed to flow through the pipe 14 and the valve 46 to the receiver 45, 40 the valve 48 will be opened to provide a vacuum and the valves 49 and 53 will be closed. Simultaneously the distillate may be discharged from the receiver 45'; for this purpose, after closing the valve 48' and opening the valve 49' the valve 45 53' is opened. When the receiver 45' is to receive the distillate and the receiver 45 is to be discharged the operation of the valves is reversed.

Instead of conveying the material to be distilled through the distillation zone by means of 50 a worm or bucket elevator, the process can also be carried out with the aid of other suitable known devices permitting the flow of the material under the influence of gravity (such as for instance stationary furnaces comprising a series 55 of hearths in step relation), or by rotation of a heated tube round its long axis (such as revolving furnaces), or by stationary furnaces provided with paddle-shaped conveying devices. It is only essential that the magnesiferous material pass through a heated zone so as to be brought to a temperature which causes transformation of the magnesium into the state of vapor, which temperature, of course, depends 60 on the pressure conditions existing in the heated system, and that, after passing through a filter, the resulting magnesium vapor is subjected to such condensation conditions that the metal will 65 be precipitated in liquid form.

In all cases, heat-resisting special steels, free from nickel and copper, must be employed for constructing the apparatus of the present invention in order to prevent contamination of the resulting magnesium. 70 75

No claim is made herein to the apparatus disclosed, this being the subject matter of a divisional application copending herewith.

I claim:—

5. 1. The process for producing substantially pure magnesium which comprises heating material containing metallic magnesium, to liberate magnesium vapor therefrom, removing the resulting vapor by a non-oxidizing gas from the heated zone, separating out dust from said vapor, and thereafter passing it into a condensation zone, and cooling it to condensation point.

10. 2. The process for producing substantially pure magnesium which comprises passing material containing metallic magnesium continuously through a heated zone under reduced pressure, to liberate magnesium vapor therefrom, removing the resulting vapor by a non-oxidizing gas from the heated zone, separating out dust from said vapor, and thereafter passing it into a condensation zone, and cooling it to condensation point.

15. 3. The process for producing substantially pure magnesium which comprises heating material containing metallic magnesium under reduced pressure to liberate magnesium vapor therefrom, removing the resulting vapor by a non-oxidizing gas from the heated zone, separating out dust from said vapor, and thereafter conveying it to a condensation zone, and cooling it to condensation point, premature condensation being prevented by keeping the vapor on its way between the distillation and condensation zone at a temperature above the solidification temperature of metallic magnesium.

20. 4. The process for producing substantially pure magnesium which comprises heating material containing metallic magnesium under reduced pressure to liberate magnesium vapor therefrom, removing the resulting vapor by a non-oxidizing gas from the heated zone, separating out dust from said vapor, and thereafter passing it into a condensation zone, and causing it to condense with intermediate liquefaction.

25. 5. The process for producing substantially pure magnesium which comprises passing material containing metallic magnesium continuously through a heated zone under reduced pressure to drive off magnesium vapor therefrom while leaving behind less volatile concomitant substances, carrying away the resulting magnesium vapor by a non-oxidizing gas from the heating zone, separating out dust from the flowing vapor, and thereafter conveying it to a condensation zone, and suddenly cooling it to condensation point.

30. 6. The process for producing substantially pure magnesium which comprises heating material containing metallic magnesium, by continuously passing the material through a heating zone under reduced pressure, nearly to the boiling point of metallic magnesium, to vaporize magnesium while leaving behind impurities not volatile at this temperature, carrying away the resulting magnesium vapor by a non-oxidizing gas from the heating zone, separating out dust from the flowing vapor, and thereafter conveying it to a condensation zone, and suddenly cooling it to condensation point, premature condensation of the magnesium vapor being prevented by keeping the mixture of non-oxidizing carrier gas and magnesium vapor on its way from the heating zone to the condensation zone, at a temperature above the solidification temperature of metallic magnesium.

35. 7. A process for separating magnesium from non-volatile concomitant substances which com-

prises passing material containing metallic magnesium continuously through a heated zone under reduced pressure to liberate magnesium vapor therefrom, carrying away the disengaged vapor by a non-oxidizing gas from the heated zone, filtering it, and thereafter passing the vapor into a condensation zone, and cooling it so as to cause it to condense with intermediate liquefaction.

40. 8. A process for separating magnesium from concomitant substances which comprises passing material containing metallic magnesium in a continuous manner through a heated zone under reduced pressure in order to heat the material to a temperature in the neighbourhood of the boiling point of metallic magnesium, carrying away the disengaged vapor by a non-oxidizing gas from the heated zone, separating out dust from the flowing vapor, and thereafter passing the vapor into a condensation zone, and suddenly cooling it to condensation point, premature condensation of the magnesium being prevented by keeping the vapor on its way between the distillation zone and the cooling zone at a temperature above the solidification temperature of metallic magnesium.

45. 9. The process for producing substantially pure magnesium which comprises heating material containing metallic magnesium under reduced pressure to liberate magnesium vapor therefrom, removing the resulting vapor from the heated zone by a non-oxidizing gas, separating dust from said vapor and thereafter passing the vapor into a condensation zone, and cooling the vapor to the condensation point.

50. 10. The process for producing substantially pure magnesium which comprises passing material containing metallic magnesium continuously in a closed system through a heated zone to liberate magnesium vapor therefrom, removing the resulting vapor by a non-oxidizing gas from the heated zone, separating dust from said vapor, thereafter passing the vapor into a condensation zone and cooling it to condensation point, and maintaining the system under reduced pressure.

55. 11. The process for producing substantially pure magnesium which comprises heating material containing metallic magnesium under reduced pressure to liberate magnesium vapor therefrom, removing the resulting vapor from the heated zone by a non-oxidizing gas, and while maintaining the system under reduced pressure separating dust from said vapor, conveying the vapor to a condensation zone maintained under reduced pressure and cooling it to condensation point, premature condensation being prevented by keeping the vapor on its way between the distillation and condensation zone at a temperature above the solidification temperature of metallic magnesium.

60. 12. The process for producing substantially pure magnesium which comprises heating material containing metallic magnesium under reduced pressure to liberate magnesium vapor therefrom, removing the resulting vapor from the heated zone by a non-oxidizing gas, and while maintaining the system under reduced pressure separating dust from said vapor, and thereafter passing it into a reduced pressure condensation zone and condensing it with intermediate liquefaction.

65. 13. The process for producing substantially pure magnesium from material containing metallic magnesium which comprises continuously passing the material in a closed system, heating the material therein nearly to the boiling point of metallic magnesium to vaporize magnesium

5

10

15

20

25

30

35

40

45

50

55

60

65

70

75

while leaving behind impurities not volatile at this temperature, carrying away the resulting magnesium vapor from the heating zone by a non-oxidizing gas, separating dust from the flowing vapor in the system, and thereafter conveying the vapor to a condensation zone in the system and suddenly cooling it to condensation point, premature condensation of the magnesium vapor being

5 prevented by keeping the mixture of non-oxidizing carrier gas and magnesium vapor on its way from the heating zone to the condensation zone at a temperature above the solidification temperature of metallic magnesium, and maintaining the system under reduced pressure. 5

FRITZ HANSGIRG.